

## UNITED STATES PATENT OFFICE

2,144,633

TREATMENT OF ARTIFICIAL FABRICS AND  
OTHER ARTIFICIAL MATERIALS

Robert Wighton Moncrieff and Frank Brentnall  
Hill, Spondon, near Derby, England, assignors  
to Celanese Corporation of America, a corpora-  
tion of Delaware

No Drawing. Application February 9, 1935, Se-  
rial No. 5,868. In Great Britain February 21,  
1934

11 Claims. (Cl. 8—130)

This invention relates to improvements in the treatment of artificial fabrics and other artificial materials, and is more particularly directed to the treatment of cellulose ester materials for the purpose of obtaining fabrics or other textile materials of improved physical properties.

The invention provides a means of improving the physical properties, particularly the handle, of materials comprising filaments, threads, ribbons or the like of organic esters of cellulose, which have been stretched and/or twisted under the influence of steam or hot water.

The materials treated may comprise yarns or the like of cellulose acetate or other organic esters of cellulose which have been subjected to treatment with steam or hot water, particularly under conditions of tension which bring about a stretching of the material, so as to produce crêpe fabrics, the treatment with the steam or hot water taking place before the application of the crêpe twist or during a single stage crêpe twisting operation or during any of the stages of a di- or multi-stage crêpe twisting operation or between any two stages of a di- or multi-stage crêpe twisting operation, as described for example in U. S. application S. No. 746,135 filed September 29, 1934, corresponding to British Patent No. 437,019, British Patent No. 438,589, U. S. application S. No. 746,134 filed September 29, 1934, corresponding to British Patent No. 438,590, U. S. application S. No. 4085 filed January 30, 1935, corresponding to British Patent No. 438,591, and U. S. application S. No. 4086 filed January 30, 1935, corresponding to British Patent No. 438,588. The materials may moreover comprise yarns or the like of cellulose acetate or other cellulose esters which have been stretched with the assistance of steam or hot water as described in U. S. applications S. Nos. 4510 and 4511 both filed February 1, 1935, corresponding to British Patents Nos. 438,584, 438,585, 438,586 and 438,587. The stretching under the influence of steam or hot water may have been applied after the whole of the crêpe twist has been inserted, for example during a bobbin to pirn winding operation or during a bobbin to bobbin winding operation.

We have now found that the physical properties, and in particular the handle, of materials by any of the above methods are substantially improved by non-superficially saponifying the cellulose ester content of the materials to a small extent. The present invention contemplates an extremely limited degree of saponification, for example so that the resultant loss in weight of a cellulose acetate material is of the order of 3 to

6%. It may be even lower or it may be somewhat higher, but preferably the loss in weight does not exceed 10%. Most advantageously the loss in weight is about 4%. With other cellulose esters saponification to an equivalent extent may be carried out or the degree of saponification may be made slightly higher as the molecular weight of the ester radicle increases. The term "non-superficially" is intended to connote that the saponification is not confined to the surface of the filaments or the like but extends to a substantial depth beneath the surface.

While the invention includes saponification with any desired saponifying agent, for example caustic soda or caustic potash, we have found that much more valuable results are obtained with saponifying agents which are somewhat slow in action or which have a substantially lower alkalinity than has caustic soda. Certain saponifying agents which have been found particularly suitable for saponifying the materials non-superficially so that a marked improvement in the physical properties, especially handle, is obtained at the expense of little loss in weight, are referred to below.

A very suitable reagent for the purpose of the invention is sodium silicate. Such a reagent may be used, for example, in aqueous solution at a concentration of about 2%, and with this concentration the desired loss in weight may be achieved by means of a treatment for about half an hour at a temperature of the order of 70–85° C. With longer times of treatment and/or higher temperatures, lower concentrations may be used, while higher concentrations will give the desired loss in weight in a shorter time or at a lower temperature. In a similar way other alkali metal salts of weak acids, and especially salts which readily form colloidal gels, e. g. sodium or potassium silicate, may be used. Again, the strong metallic bases such as caustic soda or caustic potash may be used with advantage in conjunction with gelatine or like acting substances, i. e. substances, particularly amphoteric substances, of high molecular weight, or organic colloids, capable of reducing the alkalinity of the base. Other substances which may be employed in this way, e. g. egg albumen, casein, leucine, potato starch, dextrin,  $\gamma$ -cellulose and cellobiose, are described in U. S. application S. No. 743,712 filed September 12, 1934.

Furthermore, very satisfactory results may be obtained by means of methylamine, ethylamine, ethylene diamine or similar organic bases (compare U. S. applications S. Nos. 709,335 filed Feb-

5

25

20

25

30

35

40

45

50

55

ruary 1, 1934, and 752,376 filed November 9, 1934). Thus for example one may, by treatment with a 20% solution of methylamine at 20-30° C. or of ethylene diamine at 70-80° C., obtain the desired saponification in the course of a few minutes. The saponifying action of the methylamine, ethylene diamine or similar reagent may be accelerated by means of copper or other metals or metal compounds as described in U. S. application S. No. 756,285 filed December 6, 1934.

The invention also includes the use of caustic soda, caustic potash or the like in presence of alcohols, for instance by the process described in British Patent No. 125,153 and/or in the presence of swelling agents for the cellulose derivative which do not take part in the reaction, as described in U. S. application S. No. 710,349 filed February 8, 1934.

The saponification treatment may be applied to the materials at any suitable stage after they have been subjected to the treatments described above, for example the stretching in presence of steam or hot water before, during or subsequent to crêpe twisting. Thus, the saponification may be applied before the yarn is formed into fabrics. Preferably, however, the saponification is applied subsequent to fabric formation and subsequent to the development of the crêpe figure. The invention does, however, include the saponification of materials which have been stretched in presence of steam or hot water or similar agents, quite apart from the production of crêpe fabrics.

The saponification may be carried out in any suitable manner. Most advantageously a bath treatment is employed, the fabrics or other materials being treated in such a process with a considerable volume of saponifying liquor containing the saponifying agent at the appropriate concentration and temperature. However, the materials may be saponified by other suitable processes. Methylamine, ethylene diamine and similar volatile saponifying agents may be applied to the materials in the form of vapours so as to produce the required degree of saponification.

As previously indicated, the best results are obtained by a very limited degree of saponification. The saponification may be such as just to confer upon the cellulose ester materials an affinity for cotton colours, but in most cases it will not be sufficient to reduce materially their affinity for the dispersed insoluble type of colour. Preferably in the case of using organic bases, salts such as sodium silicate or caustic soda, caustic potash or similar strong bases in presence of gelatine or like acting substances, as previously described, the extent of the saponification may be such as not to change substantially the affinity of the materials for cotton dyes or for the dispersed insoluble colours. When so treated the materials may retain all the characteristics of cellulose ester materials.

The materials treated in accordance with the invention are considerably improved in handle and particularly they are softer to the touch. The saponification does not impair the crêpe figure of the materials, which, as stated in the specifications previously referred to, is very well developed. The process of the invention is particularly important for the treatment of materials which have been very highly twisted, for example those in which the twist is of the order of 70 to 90 turns per inch or more.

What we claim and desire to secure by Letters Patent is:—

1. Process for improving the handle of materials comprising filaments, threads, ribbons and the like of organic esters of cellulose which have been stretched while being twisted under the influence of water in a fluid phase at an elevated temperature, comprising subjecting the cellulose ester content of the materials to a deep-seated saponification to an extent insufficient to impart thereto an affinity for cotton dyes.

2. Process for improving the handle of materials comprising filaments, threads, ribbons and the like of cellulose acetate which have been stretched while being twisted under the influence of water in a fluid phase at an elevated temperature, comprising subjecting the cellulose acetate content of the materials to a deep-seated saponification to an extent insufficient to impart thereto an affinity for cotton dyes.

3. Process for improving the handle of materials comprising filaments, threads, ribbons and the like of cellulose acetate which have been stretched while being twisted under the influence of water in a fluid phase at an elevated temperature, comprising subjecting the cellulose acetate content of the materials to a deep-seated saponification to an extent insufficient to impart thereto an affinity for cotton dyes by treatment in an aqueous bath of low alkalinity.

4. Process for the manufacture of artificial materials of improved handle, comprising stretching while twisting filaments, threads, ribbons or the like composed substantially of cellulose acetate, under the influence of water in a fluid phase at an elevated temperature, and subjecting the cellulose acetate content of the materials to a deep-seated saponification to an extent insufficient to impart thereto an affinity for cotton dyes by treatment in an aqueous saponifying bath of low alkalinity.

5. Process for improving the handle of materials comprising filaments, threads, ribbons and the like of organic esters of cellulose which have been stretched under the influence of water in a fluid phase at an elevated temperature, comprising subjecting the cellulose ester content of the material to deep-seated saponification to an extent insufficient to impart thereto an affinity for cotton dyes.

6. Process for improving the handle of filaments, threads, ribbons and like materials composed substantially of cellulose acetate, comprising stretching the materials under the influence of water in a fluid phase at an elevated temperature, and subjecting the cellulose acetate content of the stretched materials to deep-seated saponification without imparting thereto affinity for cotton dyes to produce loss in weight of 3 to 6% by treatment in an aqueous saponifying bath of low alkalinity.

7. Process for improving the handle of materials comprising filaments, threads, ribbons and the like of cellulose acetate which have been stretched while being twisted under the influence of water in a fluid phase at an elevated temperature, comprising subjecting the cellulose acetate content of the materials to deep-seated saponification to an extent insufficient to impart thereto an affinity for cotton dyes by treatment in an aqueous bath containing a non-aromatic organic base.

8. Process for improving the handle of materials comprising filaments, threads, ribbons and the like of cellulose acetate which have been stretched while being twisted under the influence of water in a fluid phase at an elevated tempera-

ture, comprising subjecting the cellulose acetate content of the materials to deep-seated saponification to an extent insufficient to impart thereto an affinity for cotton dyes by treatment in an aqueous bath containing a lower aliphatic amine.

5 9. Process for improving the handle of materials comprising filaments, threads, ribbons and the like of cellulose acetate which have been stretched while being twisted under the influence 10 of water in a fluid phase at an elevated temperature, comprising subjecting the cellulose acetate content of the materials to deep-seated saponification without imparting thereto an affinity for cotton dyes to produce a loss of weight of 3 to 6% 15 by treatment in an aqueous bath containing mono-methylamine.

10 10. Process for improving the handle of materials comprising filaments, threads, ribbons and the like of cellulose acetate which have been stretched while being twisted under the influence 20

of water in a fluid phase at an elevated temperature, comprising subjecting the cellulose acetate content of the materials to deep-seated saponification without imparting thereto an affinity for cotton dyes to produce a loss of weight of 3 to 6% 5 by treatment in an aqueous bath containing ethylene diamine.

11. Process for improving the handle of materials comprising filaments, threads, ribbons and the like of cellulose acetate which have been crepe 10 twisted under the influence of water in a fluid phase at an elevated temperature, comprising subjecting the cellulose acetate content of the materials to deep-seated saponification to an extent insufficient to impart thereto an affinity for 15 cotton dyes by treatment in an aqueous saponifying bath of low alkalinity.

ROBERT WIGHTON MONCRIEFF.  
FRANK BRENTNALL HILL.

20